

June 27, 1950

L. G. RAY, JR

2,512,968

MANUFACTURE OF CELLULOSIC ARTICLES

Filed April 10, 1946

2 Sheets-Sheet 1



FIG. 1.

INVENTOR.  
LINTON G. RAY JR.  
BY *Wm. J. Pritchard*  
ATTORNEY

June 27, 1950

L. G. RAY, JR

2,512,968

MANUFACTURE OF CELLULOUSIC ARTICLES

Filed April 10, 1946

2 Sheets-Sheet 2



FIG. 4.

INVENTOR.  
LINTON G. RAY JR.  
BY *Wm. V. Ditchard*  
ATTORNEY

## UNITED STATES PATENT OFFICE

2,512,968

## MANUFACTURE OF CELLULOSIC ARTICLES

Linton G. Ray, Jr., Buffalo, N. Y., assignor to  
E. I. du Pont de Nemours & Company, Wil-  
mington, Del., a corporation of Delaware

Application April 10, 1946, Serial No. 660,883

22 Claims. (Cl. 18—54)

1

This invention relates to the manufacture of regenerated cellulose articles. More particularly, it relates to improvements in the art of making high tenacity rayon from viscose.

Recently, there has been provided a method wherein viscose is extruded into a bath of such composition and maintained under such conditions as to precipitate the cellulose xanthate rapidly without substantially converting it to regenerated cellulose and, after the unregenerated structure is stretched to a marked degree, the cellulose xanthate is converted to regenerated cellulose by an appropriate treatment. The product is purified and dried, preferably while it is free from substantial tension. Though rayon yarn produced by this process is characterized by a high tensile strength and relatively low elongations, it has transverse properties which restrict the field of its utility.

An object of this invention is to provide a new and improved method for the manufacture of regenerated cellulose articles.

Another object of this invention is to provide a new and improved method for the production of rayon having improved physical characteristics.

An additional object of this invention is to provide a method of producing high tenacity rayon having improved transverse properties.

Other and additional objects of the invention will become apparent hereinafter.

The objects of the invention are accomplished, in general, by extruding viscose into a bath of such composition and maintained under such conditions as to precipitate the cellulose xanthate rapidly without substantially converting it to regenerated cellulose, stretching the unregenerated structure to a very marked degree, relaxing the unregenerated cellulose structure in the presence of a swelling solution, and then converting the cellulose xanthate to regenerated cellulose by the use of any appropriate treatment. The regenerated cellulose product is then purified and subjected to the action of a drying medium while it is preferably free from substantial tension.

Optionally, the relaxing treatment can be performed simultaneously with regeneration. The swelling bath in which the gel unregenerated (cellulose xanthate) structure is relaxed includes water as the swelling agent. Since water alone is too good a swelling agent (the cellulose xanthate of the gel unregenerated yarn under no tension will dissolve in the water), it is necessary to include a cellulose xanthate coagulant (salt) in the water. The quantity of the coagulant is such as to control and limit the swelling

2

of the yarn in the relaxed state. As will hereafter appear, the pH and the ion molality of the swelling bath must be correlated to produce the desired results.

The invention may be more readily understood by reference to the following detailed description when taken in connection with the accompanying drawings, in which:

Figure 1 is a diagrammatic side elevational view, with parts shown in section, of one form of an apparatus suitable for carrying out the invention;

Figure 2 is a diagrammatic side elevational view of a detail of a modified form of apparatus for relaxing the unregenerated gel yarns;

Figure 3 is a diagrammatic side elevational view of a detail of still another modified form of apparatus for relaxing the unregenerated gel yarns; and

Figure 4 is a graph showing the pH and ion molality range of solutions useful for swelling gel unregenerated cellulose structures.

For convenience, the invention will be described with particular reference to rayon, although in its broader aspects it is applicable to the manufacture of articles having a physical shape or form different from rayon.

Referring now to the drawings wherein like reference numerals designate like parts, the reference numeral 10 designates a candle filter to which a viscose filament-forming composition is fed in the known manner. The viscose-forming solution is forced through the candle filter 10 into and through a gooseneck 12 which is provided on the lower end thereof with a spinneret 14 positioned below the surface of the spinning bath in a tank 16. The filaments 18 issue from the spinneret 14 below the surface of the spinning bath in a tank 16 and are passed about a positively driven feed wheel 20 and cooperating freely rotatable guide roller 22, then about freely rotating rollers 24 and 26 positioned in a stretching bath in tank 28, and then about a second positively driven feed wheel 30 and cooperating freely rotatable guide roller 32. The filaments are passed about the two feed wheels 20 and 30 with a sufficient number of turns to prevent slippage of the filaments thereon so that the peripheral speeds of the respective rollers and the linear speed of the filaments thereon are the same.

Feed wheel 30 is rotated at a higher speed than feed wheel 20 so as to impart a stretch to the filaments passing through the bath in tank 28. The guide roller 32 is partially submerged in a swelling bath contained in a tank 34.

From the feed wheel 30, the yarn, wet with re-

laxing solution, drops of its own weight onto an eccentrically revolving plate 36 to build up a yarn cake 38. The eccentrically revolving plate is of the type described in United States patent to Dannenberg et al. No. 2,089,159.

Instead of applying the swelling bath to the yarn by the guide roller 32, as shown in Figure 1, a nozzle 40 can be positioned relative to the feed wheel 30 so that a swelling bath solution fed thereto will be supplied to the unregenerated cellulose filaments on such feed wheel.

Alternative to either of the previously described embodiments for subjecting the gel unregenerated filament to the swelling bath, the filaments, after leaving the feed wheel 30, can be caused to pass about a positively driven feed wheel 42 and cooperating freely rotatable guide roller 44, then about freely rotatable rollers 46 and 48 positioned in a tank 50 containing the swelling solution, and then about the feed wheel 52 and cooperating freely rotatable guide roller 54. The filaments can be passed about the feed rollers 42 and 52 with a sufficient number of turns to prevent slippage thereon. The rollers 42 and 52 are rotated at such speeds that no substantial tension is imposed on the filaments. Thus, rollers 42 and 52 can be rotated at the same speeds but, in the preferred form, the peripheral speed of roller 52 is less than the peripheral speed of roller 42 to permit yarn relaxation in the solution in tank 50. In this embodiment, the filaments, after leaving the feed wheel 52, are collected into a cake in the same manner as previously described.

The following examples illustrate certain specific embodiments of the invention, it being understood that the invention is not restricted thereto. In the examples, the parts and proportions are by weight unless otherwise specified, and the salt index is determined by the method of Reinthaler-Rowe "Artificial Silk" (1928), page 69.

#### EXAMPLE I

Viscose containing 7% cellulose, 9% sodium hydroxide and 33% carbon disulfide and having a common salt (sodium chloride) index of 4.3 was extruded through a spinneret into a bath prepared from 20% monosodium phosphate, 10% sodium sulfate and 70% water, to which was added sufficient phosphoric acid, trisodium phosphate, or both, to yield a pH of 4.1. The bath was maintained at a temperature of approximately 55° C. The filaments were passed through the bath for a distance of 6" without contact with guides or any other device which might impart tension and were then withdrawn from the bath and passed through air at normal room conditions (75° F. and atmospheric pressure) for a distance of 12" to a positively driven glass roller or feed wheel which imparted to the filaments a speed of 516" per minute. The filaments were passed around the glass roller one or more times to prevent slippage, whereby the peripheral speed of the roller and the linear speed of the filaments were approximately the same. The filaments were passed for a distance of 45" through a second bath, prepared from 18% monosodium phosphate, 2% sodium sulfate and 80% water, with the addition of sufficient phosphoric acid or trisodium phosphate, or both, to yield a pH of 4.2, after which the filaments were passed around a second positively driven glass roller which imparted a speed of 1554" per minute to the filaments. The filaments were passed one or more times about such glass roller to prevent slippage,

whereby the peripheral speed of the roller and the linear speed of the filaments were the same. Due to the speeds imparted to the filaments on the first and second positively driven rollers, the filaments were stretched during their passage through the second bath approximately three times their original length, i. e. their length at the first driven roller (the stretch thus being approximately 200%). This second bath was maintained at 100° C.

The filaments after stretching were then subjected to a relaxing bath, positioned as shown in Figure 1 of the drawings, prepared from 12% sodium sulfate and 88% water. Such bath, which had a pH of 7 and an ion molality of 2.9, was maintained at room temperature (75° F. and atmospheric pressure). The yarn, upon leaving the second positively driven roller and while wet with the relaxing solution, was allowed to fall of its own weight onto a flat plate which was so moved as to traverse the yarn according to any desired pattern and thus build up a suitable cake or package. The filaments or yarn at this point were still in the form of cellulose xanthate free from any substantial degree of regeneration. The cake was then covered with a cloth wrapping and immersed for a period of 16 hours in a solution at 55° C. having the same composition as the first or spinning bath to convert the yarn to regenerated cellulose. The cake was removed from the regenerating bath. After being washed free of occluded salts, it was treated with a lubricating finish and was dried.

A comparison of the properties of yarn produced by this procedure and of yarn produced by the identical procedure except that the treatment with the relaxing bath is omitted (designated as "Control") is set forth hereafter in Table A.

#### EXAMPLE II

Viscose containing 5.1% cellulose, 9.1% sodium hydroxide and 23.5% carbon disulfide and having a common salt (sodium chloride) index of 2.0 was extruded through a spinneret into a bath prepared from 22.3% monosodium phosphate, 9.1% sodium sulfate and 68.6% water, to which was added sufficient phosphoric acid, trisodium phosphate, or both, to yield a pH of 3.5. The bath was maintained at a temperature of approximately 55° C. The filaments were passed through the bath for a distance of 6" without contact with guides or any other device which might impart tension and were then withdrawn from the bath and passed through air at normal room conditions (75° F. and atmospheric pressure) for a distance of 14" to a positively driven glass roller or feed wheel which imparted to the filaments a speed of 450" per minute. The filaments were passed around the glass roller one or more times to prevent slippage, whereby the peripheral speed of the roller and the linear speed of the filaments were approximately the same. The filaments were passed for a distance of 40" through a second bath, prepared from 18% monosodium phosphate, 2% sodium sulfate and 80% water, with the addition of sufficient phosphoric acid or trisodium phosphate, or both, to yield a pH of 6.5, after which the filaments were passed around a second positively driven glass roller which imparted a speed of 1636" per minute to the filaments. The filaments were passed one or more times about such glass roller to prevent slippage, whereby the peripheral speed of the roller and the linear speed were approximately the same. Due to the speeds imparted to the

filaments on the first and second positively driven rollers, the filaments were stretched during their passage through the second bath approximately 3.75 times their original length, i. e. their length at the first driven roller (the stretch thus being approximately 275%). This second bath was maintained at 100° C.

The filaments after stretching were then subjected to a relaxing bath, positioned as shown in Figure 1 of the drawings, prepared from 11% sodium sulfate and 89% water. Such bath, which had a pH of 7 and an ion molality of 2.6, was maintained at room temperature (75° F. and atmospheric pressure). The yarn, upon leaving the second positively driven roller and while wet with the relaxing solution, was allowed to fall of its own weight onto a flat plate which was so moved as to traverse the yarn according to any desired pattern and thus build up a suitable cake or package. The filaments or yarn at this point were still in the form of cellulose xanthate free from any substantial degree of regeneration. The cake was then covered with a cloth wrapping and immersed for a period of 30 minutes in a boiling solution, having the same composition as the first or spinning bath but adjusted to a pH of 5, to convert the yarn to regenerated cellulose. The cake was removed from the regenerating bath. After being washed free of occluded salts, it was treated with a lubricating finish and was dried.

A comparison of the properties of yarn produced by this procedure and of yarn produced by the identical procedure except that the treatment with the relaxing bath is omitted (designated as "Control") is set for hereinafter in Table A.

### EXAMPLE III

Viscose containing 7% cellulose, 9.1% sodium hydroxide and 33% carbon disulfide and having a common salt (sodium chloride) index of 4.5 was extruded through a spinneret into a bath prepared from 20% monosodium phosphate, 10% sodium sulfate and 70% water, to which was added sufficient phosphoric acid, trisodium phosphate, or both, to yield a pH of 4.0. The bath was maintained at a temperature of approximately 55° C. The filaments were passed through the bath for a distance of 6" without contact with guides or any other device which might impart tension and were then withdrawn from the bath and passed through air at normal room conditions (75° F. and atmospheric pressure) for a distance of 14" to a positively driven glass roller or feed wheel which imparted to the filaments a speed of 450" per minute. The filaments were passed around the glass roller one or more times to prevent slippage, whereby the peripheral speed of the roller and the linear speed of the filaments were approximately the same. The filaments were passed for a distance of 40" through a second bath, prepared from 18% monosodium phosphate, 2% sodium sulfate and 80% water, with the addition of sufficient phosphoric acid or trisodium phosphate, or both, to yield a pH of 3.8 to 4.2, after which the filaments were passed around a second positively driven glass roller which imparted a speed of 1473" per minute to the filaments. The filaments were passed one or more times about such glass roller to prevent slippage, whereby the peripheral speed of the roller and the linear speed were approximately the same. Due to the speeds imparted to the filaments on the first and second positively driven rollers, the filaments were stretched during their passage through the second bath approximately 75

3.23 times their original length, i. e. their length at the first driven roller (the stretch thus being approximately 223%). This second bath was maintained at 100° C.

5 The filaments after stretching were then subjected to a relaxing bath, positioned as shown in Figure 1 of the drawings, prepared from 11% sodium sulfate and 89% water. Such bath, which had a pH of 7 and an ion molality of 2.6, was maintained at room temperature (75° F. and atmospheric pressure). The yarn, upon leaving the second positively driven roller and while wet with relaxing solution, was allowed to fall of its own weight onto a flat plate which was so moved as to traverse the yarn according to any desired pattern and thus build up a suitable cake or package. The filaments or yarn at this point were still in the form of cellulose xanthate free from any substantial degree of regeneration. The cake was then covered with a cloth wrapping and immersed for a period of 30 minutes in a boiling solution, having the same composition as the first or spinning bath but adjusted to a pH of 5, to convert the yarn to regenerated cellulose. 10 The cake was removed from the regenerating bath. After being washed free of occluded salts, it was treated with a lubricating finish and was dried.

30 A comparison of the properties of yarn produced by this procedure and of yarn produced by the identical procedure except that the treatment with the relaxing bath is omitted (designated as "Control") is set forth hereafter in Table A.

### EXAMPLE IV

Viscose containing 5% cellulose, 9% sodium hydroxide and 30% carbon disulfide and having a common salt (sodium chloride) index of 5.0 was extruded through a spinneret into a bath prepared from 20% monosodium phosphate, 10% sodium sulfate and 70% water, to which was added sufficient phosphoric acid, trisodium phosphate, or both, to yield a pH of 3.0. The bath was maintained at a temperature of approximately 60° C. The filaments were passed through the bath for a distance of 6" without contact with guides or any other device which might impart tension and were then withdrawn from the bath and passed through air at normal room conditions (75° F. and atmospheric pressure) for a distance of 14" to a positively driven glass roller or feed wheel which imparted to the filaments a speed of 450" per minute. The filaments were passed around the glass roller one or more times to prevent slippage, whereby the peripheral speed of the roller and the linear speed of the filaments were approximately the same. The filaments were passed for a distance of 40" in the air at normal room conditions (75° F. and atmospheric pressure) and thence around a second positively driven roller which imparted a speed of 1453" per minute. The filaments were passed one or more times about such roller to prevent slippage whereby the peripheral speed of the roller and the linear speed were approximately the same. Due to the speeds imparted to the filaments on the first and second positively driven rollers, the filaments were stretched in air approximately 3.20 times their original length, i. e. their length at the first driven roller (the stretch thus being approximately 220%).

70 The filaments after stretching were then subjected to a relaxing bath, positioned as shown in Figure 3 of the drawings, prepared from 15%

sodium sulfate, 2% sodium hydroxide and 83% water. Such bath, which had a pH of 10.9 and an ion molality of 4.4, was maintained at room temperature (75° F. and atmospheric pressure). The yarn was withdrawn from the relaxing bath by a roller which imparted a speed of 1453" per minute to the yarn and, while wet with relaxing solution, was allowed to fall of its own weight onto a flat plate which was so moved as to traverse the yarn according to any desired pattern and thus build up a suitable cake or package. The filaments or yarn at this point were still in the form of cellulose xanthate free from any substantial degree of regeneration. The yarn was regenerated and processed normally.

A comparison of the properties of yarn produced by this procedure and of yarn produced by the identical procedure except that the treatment with the relaxing bath is omitted (designated as "Control") is set forth hereafter in Table A.

5 phosphate, or both, to yield a pH of 4.1, after which the filaments were passed around a second positively driven glass roller which imparted a speed of 1566" per minute to the filaments. The filaments were passed one or more times about the second roller to prevent slippage, whereby the peripheral speed of such roller and the linear speed of the filaments were the same. Due to the linear speeds imparted to the filaments on the 10 first and second positively driven rollers, the filaments were stretched through the second bath approximately 3.48 times their original length, i. e. their length at the first driven roller (the stretch thus being approximately 248%). The second bath was maintained at 100° C.

15 The filaments, upon leaving the second positively driven roller, were allowed to fall of their own weight onto a flat plate, as is set forth in Example I. The filaments or yarns at this point were still in the form of cellulose xanthate free from any substantial degree of regeneration. The

Table A

|             | Relaxing Bath                                  |      |              | Denier | Filament | Tenacity |      |      | Elongation |      |      | Ratios           |                  |
|-------------|------------------------------------------------|------|--------------|--------|----------|----------|------|------|------------|------|------|------------------|------------------|
|             | Coagulant                                      | pH   | Ion Molality |        |          | Dry      | Wet  | Loop | Dry        | Wet  | Loop | W/D <sup>1</sup> | L/D <sup>2</sup> |
| Control     |                                                |      |              | 257    | 150      | 4.90     | 3.57 | 2.61 | 6.2        | 7.2  | 3.2  | 0.73             | 0.53             |
| Example I   | Na <sub>2</sub> SO <sub>4</sub>                | 7    | 2.9          | 285    | 150      | 4.60     | 3.24 | 3.26 | 8.4        | 10.3 | 5.3  | 0.70             | 0.71             |
| Control     |                                                |      |              | 262    | 150      | 5.61     | 4.14 | 2.98 | 7.3        | 7.5  | 3.7  | 0.74             | 0.53             |
| Example II  | Na <sub>2</sub> SO <sub>4</sub>                | 7    | 2.6          | 276    | 150      | 5.14     | 3.88 | 3.43 | 8.2        | 9.0  | 5.0  | 0.76             | 0.67             |
| Control     |                                                |      |              | 281    | 200      | 5.82     | 4.12 | 3.20 | 6.9        | 7.5  | 3.7  | 0.71             | 0.55             |
| Example III | Na <sub>2</sub> SO <sub>4</sub>                | 7    | 2.6          | 292    | 200      | 5.38     | 3.87 | 3.48 | 7.2        | 8.4  | 4.3  | 0.72             | 0.65             |
| Control     |                                                |      |              | 282    | 200      | 5.44     | 4.16 | 3.36 | 8.8        | 10.0 | 5.1  | 0.76             | 0.62             |
| Example IV  | 15% Na <sub>2</sub> SO <sub>4</sub><br>2% NaOH | 10.9 | 4.4          | 290    | 200      | 5.26     | 3.76 | 3.58 | 10.7       | 12.0 | 6.5  | 0.71             | 0.67             |

<sup>1</sup> W/D = wet tenacity  
dry tenacity.

<sup>2</sup> L/D = loop tenacity  
dry tenacity.

In the preferred embodiment of the invention as shown by the foregoing examples, the filaments or yarns were subjected to the treatment with the relaxing solution prior to regeneration and while the filaments or yarns were in substantially the unregenerated gel form and consisted essentially of water-soluble cellulose xanthate. However, the relaxation can be combined with regeneration, as shown by the following examples:

#### EXAMPLE V

Viscose containing 5% cellulose, 9% sodium hydroxide and 23.5% carbon disulfide and having a common salt (sodium chloride) index of about 2.2 was extruded through a spinneret into a bath prepared from 20% monosodium phosphate, 10% sodium phosphate and 70% water, to which was added sufficient phosphoric acid, trisodium phosphate, or both, to yield a pH of 4.2. The bath was maintained at a temperature of approximately 55° C. The filaments were passed through the bath for a distance of 5" without contact with guides or any other device which might impart tension and passed through air at normal room conditions (75° F. and atmospheric pressure) for a distance of 12" to a positively driven glass roller or feed wheel which imparted to the filaments a speed of 450" per minute. The filaments were passed around the glass roller one or more times to prevent slippage whereby the peripheral speed of the roller and the linear speed of the filaments were approximately the same. The filaments were passed for a distance of 40" through a second bath prepared from 18% monosodium phosphate, 2% sodium sulfate and 80% water, with the addition of sufficient phosphoric acid or trisodium

40 phosphate, or both, to yield a pH of 4.9 and an ion molality of 2.8, whereby the yarn was simultaneously relaxed and regenerated:

Per cent

Sodium sulfate ..... 3.5  
Monosodium phosphate ..... 9.0  
Water ..... 87.5

Sufficient sodium hydroxide was added to the bath to raise the pH to 4.9.

50 The cake was removed from the bath and, after being washed free of occluded salts, it was treated with a lubricating finish and dried.

55 A comparison of yarn produced by this procedure and of yarn produced by the identical procedure except that the yarn was regenerated in the following bath having a pH of 4.5 and an ion molality of 5.1 (designated as "Control") is hereinafter set forth in Table B:

Per cent

Sodium sulfate ..... 6  
Monosodium phosphate ..... 15  
Water ..... 79

Sufficient sodium hydroxide was added to the bath to raise the pH to 4.5.

#### EXAMPLE VI

65 Same as Example V, except that the relaxing and regenerating bath, consisting of the following ingredients, had a pH of 5.0 and an ion molality of 1.7.

Per cent

Sodium sulfate ..... 2  
Monosodium phosphate ..... 6  
Water ..... 92

Sufficient sodium hydroxide was added to the bath to raise the pH to 5.0.

A comparison of the properties of the yarn produced by this procedure and of yarn produced by the identical procedure except that the yarn was only regenerated in the following bath having a pH of 4.5 and an ion molality of 5.1 (designated as "Control") is hereinafter set forth in Table B:

|                      | Per cent |
|----------------------|----------|
| Sodium sulfate       | 6        |
| Monosodium phosphate | 15       |
| Water                | 79       |

Sufficient sodium hydroxide was added to the bath to raise the pH to 4.5.

limit of optimum concentration at these high pH values is limited by the solubility of the salt under consideration.

The graph constituting Figure 4 of the drawings shows the relationship of the ion molality and pH of the solution. As shown by the curves of Figure 4, to be effective for the invention the aqueous solution also has an ion molality within the limits defined by the curves AB and CD, and preferably within the limits defined by the curves EF and GH, and the pH at the point on the ordinate of the graph corresponding to said ion molality.

In the preferred embodiment of the invention,

Table B

|            | Relaxing Bath                                                                             |     |              | Denier | Filament | Tenacity |      |      | Elongation |     |      | Ratios           |                  |      |
|------------|-------------------------------------------------------------------------------------------|-----|--------------|--------|----------|----------|------|------|------------|-----|------|------------------|------------------|------|
|            | Coagulant                                                                                 | pH  | Ion Molality |        |          | Dry      | Wet  | Loop | Dry        | Wet | Loop | W/D <sup>1</sup> | L/D <sup>2</sup> |      |
| Control    | {(Na <sub>2</sub> SO <sub>4</sub> )<br>(NaH <sub>2</sub> PO <sub>4</sub> )}               | 4.5 | 5.1          | 136    |          | 100      | 5.28 | 4.42 | 2.32       | 5.7 | 6.9  | 2.0              | 0.84             | 0.44 |
| Example V  | {(Na <sub>2</sub> SO <sub>4</sub> )<br>(Na <sub>2</sub> H <sub>2</sub> PO <sub>4</sub> )} | 4.9 | 2.8          | 140    |          | 100      | 4.83 | 3.79 | 2.76       | 6.9 | 8.1  | 3.3              | 0.79             | 0.57 |
| Example VI | {(Na <sub>2</sub> SO <sub>4</sub> )<br>(Na <sub>2</sub> H <sub>2</sub> PO <sub>4</sub> )} | 5.0 | 1.7          | 156    |          | 100      | 3.77 | 3.12 | 2.81       | 9.4 | 11.5 | 5.9              | 0.83             | 0.75 |

<sup>1</sup> W/D = wet tenacity.  
dry tenacity.

<sup>2</sup> L/D = loop tenacity.  
dry tenacity.

Though it is preferred to employ aqueous solutions of sodium sulfate as the relaxing bath, it is to be understood that the invention is not restricted to such bath. In general, an aqueous solution of any water-soluble salt which will precipitate or coagulate viscose without substantial regeneration can be used. As illustrative examples of salts other than sodium sulfate which can be used are ammonium sulfate, ammonium chloride, ammonium carbonate, sodium phosphate, etc., or mixtures thereof, and with or without an alkali. In the claims, the expression "an aqueous solution of a water-soluble salt which is a coagulant for cellulose xanthate" is intended to define a solution containing such a salt or mixtures of such salts and with or without an alkali.

It is assumed that the effect of the dilute salt baths on the swelling of the unregenerated gel yarns is primarily a function of the molality of the ion present. However, since the hydroxyl ion exerts a specific swelling action on cellulose, the molality of the swelling bath must be increased when above a pH of 7 to counterbalance the swelling action of the hydroxyl ion. The molality of the solution is calculated as the number of gram ions per 1000 grams of solvent, assuming 100% ionization but disregarding the presence of hydrogen or hydroxyl ions.

Experiments have shown that for an aqueous relaxing solution of a neutral salt at an approximate pH of 7, the preferable range of molality is between 2 and 3, with some definite beneficial effect between the molality of 1 and 4. Below a molality of 1, excessive swelling and incipient solution occur, and above a molality of 4 little effect is observed. Experiments have also shown that as the pH is increased above 7, as, for example, by addition of alkali hydroxide, the molality of the solution must be increased about 0.5 unit for every two unit change in pH so that at a pH of, for example, 11, the minimum useful range starts at a molality of 2 and the optimum range at a molality of 3. The upper limits of the optimum range broadens considerably at higher pHs, so that at a pH of 10 a molality of as high as 5 gives good effects. It is probable that the upper

30 the relaxing bath consists of an aqueous solution of sodium sulfate having concentrations of from 9% to 13%.

35 The following aqueous solutions, containing the named coagulant and having the ion molality and pH values set forth in the following Table C, have also produced satisfactory results as relaxing solutions in the method herein described:

Table C

| 40                                                     | Coagulant | pH    | Ion Molality |
|--------------------------------------------------------|-----------|-------|--------------|
| Na <sub>2</sub> SO <sub>4</sub>                        |           | 7.0   | 1.59         |
| Do                                                     |           | 7.0   | 2.51         |
| Do                                                     |           | 7.0   | 3.72         |
| (NH <sub>4</sub> ) <sub>2</sub> SO <sub>4</sub>        |           | 5.0   | 1.59         |
| Do                                                     |           | 5.0   | 2.51         |
| Do                                                     |           | 5.0   | 3.72         |
| NaCl                                                   |           | 7.0   | 1.59         |
| Do                                                     |           | 7.0   | 2.51         |
| Do                                                     |           | 7.0   | 3.72         |
| Na <sub>2</sub> CO <sub>3</sub>                        |           | 10.6  | 3.14         |
| Do                                                     |           | 10.0  | 5.03         |
| Na <sub>2</sub> PO <sub>4</sub>                        |           | 11.25 | 2.71         |
| Na <sub>2</sub> SO <sub>4</sub> +2% Na <sub>2</sub> OH |           | 10.8  | 3.75         |
| Na <sub>2</sub> SO <sub>4</sub> +NaOH                  |           | 9.2   | 3.17         |

55 The means by which the unregenerated stretched yarn is subjected to the relaxing bath is not limited to those herein described. If desired, immersion of trays of the relaxed unregenerated yarn in the swelling bath can be used. Also, the relaxing solution can be applied by both the dip bath of Figure 1 and the drip bath of 60 Figure 2. The gel unregenerated yarn at the time it is treated with the relaxing bath or while wet with the relaxing solution is preferably in a substantially tension-free state.

The duration of treatment with the relaxing bath is not critical and may vary from 5 seconds to 1 hour or more.

70 The coagulating baths utilized in the above examples under the conditions present exert a strong and rapid coagulating effect on viscose without at the same time causing any substantial degree of regeneration of the coagulated xanthate structure. The pH of the coagulating bath is maintained within the range of 3.0 to 7.0 and preferably within the range of 3.5 to 5.5, and the coagulating bath contains 10% or more of phos-

## 11

phate ion, calculated for convenience as trisodium phosphate, i. e., although all of the phosphate radical is not necessarily present in the form of trisodium phosphate, nevertheless in stating that the coagulating bath liquid contains 10% or more by weight of phosphate, this signifies a weight calculation on the convenient assumption that all of the phosphate is present as trisodium phosphate. It is obvious that the phosphate radical may be present in other forms, for example in the form of mono- or disodium phosphates; or other soluble phosphates, for example the phosphates of alkali metals other than sodium. Also, other phosphates such as ammonium phosphate, organic amine phosphates and the like can be used. However, because of the greater efficiency of the alkali metal phosphates in the practice of the invention and their lesser cost, alkali metal phosphates are preferred.

In describing the specific composition of the phosphate baths utilized in the above examples, it is to be understood that although the baths can be made up from commercially available materials so as to have approximately the desired pH, nevertheless it is usually advisable to add a certain amount of phosphate, e. g. phosphoric acid or its salts, so as to adjust the pH of the bath accurately to the desired value. Also, it is not necessary for the aqueous composition initially utilized in making up the bath to possess a pH close to that desired since, by the addition of the proper amount of whatever phosphate is needed, the desired pH can be attained.

The above examples utilize coagulating baths in which the phosphate is present largely, if not entirely, in the form of monosodium phosphate. The use of alkali metal phosphates is preferred, and the greater utility of the alkali metal phosphates is based, at least in part, on the fact that the mono- and disodium phosphates existing as such under the pH conditions prevailing in the coagulating bath, and being salts of a strong base and a weak acid (the second and third hydrogen atoms of phosphoric acid having a low degree of ionization), exhibit a buffering action in the bath, i. e. relatively large amounts of the alkali carried over in the viscose can be neutralized without markedly changing the pH of the bath. Other similar buffering agents such as sodium acetate can, if desired, be added to supplement the buffering action of the phosphate salts. This buffering characteristic makes possible the rapid and uniform coagulation of the viscose due to the substantially constant pH conditions of the bath over relatively long periods of use. By contrast, previously known coagulating baths consisting of aqueous solutions of ammonium sulfate (which have a pH of less than 7.0) exhibit no buffering action.

Although the coagulating bath can comprise, if desired, an aqueous solution containing only an alkali metal salt of phosphoric acid in an amount of 10% and preferably 15% or more by weight, in addition to the phosphate, the bath may also contain salts of strong acids. Thus, as indicated in Example I, the bath may also contain sodium sulfate, one typical form of such bath being an aqueous solution containing 20% monosodium phosphate and from 2% to 20% of sodium sulfate, the bath being adjusted to a pH of, for example, 4.0 to 4.5. Another material that can be added to the phosphate baths with advantage is ammonium sulfate.

The coagulating bath is preferably maintained at a temperature of 45° to 75° C., the yarn travel

## 12

through the bath preferably being of the order of 2 inches to 18 inches. However, these temperatures and bath travels are not critical, provided only that they are not so great as to cause any substantial degree of regeneration of the cellulose xanthate structures produced therein. The yarn must, however, be preferably completely coagulated before it is subjected to the subsequent stretching operation of the invention. When the travel through the coagulating bath is insufficient to completely coagulate the extruded viscose, it is desirable to lag the incompletely coagulated yarn under low tension, for example by passing it through air, for a time sufficient to complete the coagulation. Or, if desired, the yarn can be passed through a second phosphate coagulating bath for a period of time sufficient to complete the coagulation. If the yarn is not completely coagulated prior to stretching, the amount of stretch obtainable will be distinctly impaired.

When the coagulating bath is rendered unfit for further use because of the addition of large amounts of caustic from the viscose solution, it can be reconditioned for further use by the addition of fresh amounts of phosphoric acid. It can also be reconditioned by the addition of sufficient sulfuric acid to make the total sulfate ion content substantially equivalent to the total sodium ion content of the bath, the solution then being concentrated by evaporation and strongly cooled (to 0° C.) to crystallize out sodium sulfate. The remaining concentrated solution of phosphoric acid can then be used to strengthen or recondition further volumes of waste bath.

It is important for coagulation to take place under conditions of very low tension. Thus, the tension imposed on the filaments in the coagulating bath should not be in excess of 0.1 gram per denier and preferably not in excess of 0.01 gram per denier. Where the viscose structure is non-filamentary, tensions equivalent to those given in connection with filaments will be used.

The stretching of the coagulated-only yarn can be accomplished by passing the yarn about positively driven pairs of stretching rolls or in any other known manner. In accordance with the examples, this stretching is preferably performed while the yarn is passing through a bath of the same general type as the coagulating bath, but heated almost to the boil since such baths assist in developing the greatest degree of stretch. However, this is not essential. The stretching operation can, if desired, be performed in the presence of an aqueous solution of inorganic salts, a liquid such as glycerin, triethanolamine, ethylene glycol, etc., or even in the presence of a gaseous medium such as live steam, air, carbon dioxide, sulfur dioxide, etc. These stretching media are preferably maintained at an elevated temperature, for example 100° C. or more. However, this is not critical to the practice of the invention and they can, if desired, be maintained at any other temperature, for example at room temperature. In accordance with the principles of this invention, the yarn at the start of the stretching operation is substantially unregenerated and is water-soluble. The duration of the stretching operation and the contact of the yarn with the stretching medium is preferably so short that no substantial amount of regeneration is effected.

The stretched relaxed yarn is collected in suitable package form and regenerated. It may be collected on a rotating bobbin in the form of a

cross-wound package or in a centrifugal bucket of the type customarily employed in the spinning of viscose rayon yarn, or it may be collected in any other package form. Preferably, however, the yarn is permitted to fall in a relaxed, tensionless state on to a slowly moving support and formed into a cake-like package in the manner of Example I above. The yarn package protected by a suitable cover is then treated with a regenerating bath for a suitable period of time. This bath can comprise a mineral acid solution, for example of the type generally employed in the single bath process in the spinning of viscose rayon yarn and containing from 8% to 10% sulfuric acid, together with varying amounts of inorganic salts such as sodium sulfate, etc., or it may comprise an aqueous inorganic salt solution or an inert liquid (such as glycerin) heated to a high temperature. Preferably, however, it comprises a boiling solution of the same general type as the coagulating or stretching baths. On the other hand, the yarn wet with occluded coagulating bath and stretching bath liquors can be regenerated by spontaneous decomposition of the cellulose xanthate by permitting it to stand a sufficiently long time (for example 24 hours) at room temperature. In such a case, of course, the humidity of the surrounding atmosphere should be maintained sufficiently high to prevent crystallization within the yarn of those salts contained in the occluded liquors.

It is not necessary that the yarn be regenerated and purified in package form. The coagulated-only yarn can be led through a regenerating bath in a continuous manner prior to its collection in package form, or the yarn can be collected in a tensionless manner on a slowly moving conveyor belt of the type shown in British Patent No. 379,880 to Topham, the yarn collected in the form of small overlapping ringlets being subsequently led under showers of regenerating and purifying liquids and dried.

Although any method can be used in preparing the viscose utilized in the practice of the invention, the viscose employed in the examples was prepared by a standard method involving the combination of alkali (soda) cellulose with the percentage of carbon bisulfide (recited in the examples) based on the cellulose content of the alkali cellulose. Also, viscoses having a wide range of viscosities may be used, but it is preferred that viscoses which have been submitted to a very short ripening period and have a salt index of about 2.0 to 2.5 be spun. The use of the strong coagulating baths of this invention causes rapid coagulation of such viscoses. It is also preferred, although not critical, that the alkali cellulose used be subjected only to a short aging period.

It is preferred, in order to develop the greatest stretchability of the coagulated, unregenerated structures, to utilize viscose in which the caustic content is higher than the cellulose content, e. g. a viscose containing 7% cellulose and 9% sodium hydroxide. However, other viscoses which have a sodium hydroxide content less than the cellulose may also be used and, generally speaking, viscoses having a cellulose or caustic content of between 4% and 9%, or more, are quite satisfactory.

The invention can be applied to continuous spinning, purification and collection processes of any character.

In carrying out the invention, it is possible to produce either straight or crimped filaments.

For example, where the coagulating baths contain, in addition to phosphates, a high concentration, e. g. 20%, of ammonium sulfate or of sodium sulfate, or both, then filaments are produced which have a good permanent crimp or which develop a good permanent crimp when treated in a state free of substantial tension with water or dilute aqueous caustic soda. If the stretched yarn is regenerated in a state free of substantial tension, even though tension is applied during the subsequent steps of washing and drying, the yarn develops a decided degree of crimp upon treatment with hot water or dilute caustic soda. Also, even though tension is used during regeneration and subsequent purification and drying treatments and thereby acquires no crimp, nevertheless, it will develop a very good permanent crimp upon being treated in a relaxed state in hot water or dilute caustic solution.

As is shown by the above tables, the transverse properties of the rayon treated in accordance with this invention are materially improved. This is indicated by the improved loop tenacity without marked loss in dry tenacity.

As is shown by the tables, yarn prepared by the preferred sodium sulfate relaxation have generally improved loop strengths (up to 0.5 to 0.6 gram per denier greater than the controls), decreased wet and dry tenacities (losses of approximately 0.5 gram denier in each), and greater wet, dry and loop elongations than rayon spun by identical processes but omitting the relaxation treatment.

The relaxed yarns are considerably less brittle than yarns prepared by identical processes except that the relaxing treatment is omitted. As a general rule the yarns of this invention are duller in appearance and appear to show a tendency toward waviness. The improved properties of the yarn of this invention become apparent from the following table:

Table D

|                                                   | Den./Fil. | Number of Flexes to Failure <sup>1</sup> |
|---------------------------------------------------|-----------|------------------------------------------|
| Yarn with relaxing treatment of this invention    | 1.42      | 1,450                                    |
| Yarn without relaxing treatment of this invention | 1.35      | 450                                      |

<sup>1</sup> Determined on Masland flex tester.

The invention not only makes it possible to produce a yarn of very desirable properties, but also makes possible a spinning process that is admirably adapted for use on a commercial scale. The process does not require the use of complicated apparatus or difficultly prepared baths.

The invention has its principal utility in the manufacture of filaments and yarns. However, the invention, broadly speaking, is applicable also to the production of thin tubing and other types of products by the viscose process with the attaining of generally the same advantages which result from the use of the invention in the manufacture of filaments and yarns.

Since the operation of the invention as described above is capable of considerable modification, any variation which conforms to the spirit of the invention is intended to be included within the claims.

I claim:

1. In the process for the production of a regenerated cellulose structure which comprises ex-

## 15

truding viscose into a coagulating bath which will precipitate the cellulose xanthate without substantially converting it to regenerated cellulose, drawing said structure from said bath, stretching said structure and regenerating the same to regenerated cellulose, the improvement which comprises the step of swelling the structure subsequent to stretching in the presence of an aqueous solution of a water-soluble salt which is a coagulant for cellulose xanthate, said solution having an ion molality within the limits defined by the curves AB and CD of the graph shown as Figure 4 in the accompanying drawings and the pH at the point on the ordinate of said graph corresponding to said ion molality.

2. In the process for the production of a regenerated cellulose structure which comprises extruding viscose into a coagulating bath which will precipitate the cellulose xanthate without substantially converting it to regenerated cellulose, drawing said structure from said bath, stretching said structure and regenerating the same to regenerated cellulose, the improvement which comprises the step of swelling the structure subsequent to stretching and prior to regeneration in the presence of an aqueous solution of a water-soluble salt which is a coagulant for cellulose xanthate, said solution having an ion molality within the limits defined by the curves AB and CD of the graph shown as Figure 4 in the accompanying drawings and the pH at the point on the ordinate of said graph corresponding to said ion molality.

3. In the process for the production of a regenerated cellulose structure which comprises extruding viscose into a coagulating bath which will precipitate the cellulose xanthate without substantially converting it to regenerated cellulose, drawing said structure from said bath, stretching said structure and regenerating the same to regenerated cellulose, the improvement which comprises the step of swelling the structure subsequent to stretching and simultaneously with regeneration in the presence of an aqueous solution of a water-soluble salt which is a coagulant for cellulose xanthate, said solution having an ion molality within the limits defined by the curves AB and CD of the graph shown as Figure 4 in the accompanying drawings and the pH at the point on the ordinate of said graph corresponding to said ion molality.

4. In the process for the production of a regenerated cellulose structure which comprises extruding viscose into a coagulating bath which will precipitate the cellulose xanthate without substantially converting it to regenerated cellulose, drawing said structure from said bath, stretching said structure and regenerating the same to regenerated cellulose, the improvement which comprises the step of swelling the structure subsequent to stretching in the presence of an aqueous solution of a water-soluble salt which is a coagulant for cellulose xanthate, said solution having an ion molality within the limits defined by the curves EF and GH of the graph shown as Figure 4 in the accompanying drawings and the pH at the point on the ordinate of said graph corresponding to said ion molality.

5. In the process for the production of a regenerated cellulose structure which comprises extruding viscose into a coagulating bath which will precipitate the cellulose xanthate without substantially converting it to regenerated cellulose, drawing said structure from said bath, stretching said structure and regenerating the

## 16

same to regenerated cellulose, the improvement which comprises the step of swelling the structure subsequent to stretching and prior to regeneration in the presence of an aqueous solution of a water-soluble salt which is a coagulant for cellulose xanthate, said solution having an ion molality within the limits defined by the curves EF and GH of the graph shown as Figure 4 in the accompanying drawings and the pH at the point on the ordinate of said graph corresponding to said ion molality.

6. In the process for the production of a regenerated cellulose structure which comprises extruding viscose into a coagulating bath which will precipitate the cellulose xanthate without substantially converting it to regenerated cellulose, drawing said structure from said bath, stretching said structure and regenerating the same to regenerated cellulose, the improvement which comprises the step of swelling the structure subsequent to stretching and simultaneously with regeneration in the presence of an aqueous solution of a water-soluble salt which is a coagulant for cellulose xanthate, said solution having an ion molality within the limits defined by the curves EF and GH of the graph shown as Figure 4 in the accompanying drawings and the pH at the point on the ordinate of said graph corresponding to said ion molality.

7. In the process for the production of a regenerated cellulose structure which comprises extruding viscose into a coagulating bath which will precipitate the cellulose xanthate without substantially converting it to regenerated cellulose, drawing said structure from said bath, stretching said structure and regenerating the same to regenerated cellulose, the improvement which comprises the step of swelling the structure subsequent to stretching in the presence of an aqueous solution of a water-soluble neutral salt which is a coagulant for cellulose xanthate, said solution having an ion molality of from 1 to 4 and a pH of 7.

8. In the process for the production of a regenerated cellulose structure which comprises extruding viscose into a coagulating bath which will precipitate the cellulose xanthate without substantially converting it to regenerated cellulose, drawing said structure from said bath, stretching said structure and regenerating the same to regenerated cellulose, the improvement which comprises the step of swelling the structure subsequent to stretching in the presence of an aqueous solution of a water-soluble neutral salt which is a coagulant for cellulose xanthate, said solution having an ion molality of from 2 to 3 and a pH of 7.

9. In the process for the production of a regenerated cellulose structure which comprises extruding viscose into a coagulating bath which will precipitate the cellulose xanthate without substantially converting it to regenerated cellulose, drawing said structure from said bath, stretching said structure and regenerating the same to regenerated cellulose, the improvement which comprises the step of swelling the structure subsequent to stretching in the presence of an aqueous solution having a pH of 7 and an ion molality of from 1 to 4 and consisting of water and sodium sulfate, the latter being present in an amount of from 9% to 13% by weight of the solution.

10. In the process for the production of a regenerated cellulose yarn which comprises extruding viscose filaments into a coagulating bath which will precipitate the cellulose xanthate

without substantially converting it to regenerated cellulose, drawing said filaments from said bath, stretching said filaments and regenerating said filaments to regenerated cellulose, the improvement which comprises the step of swelling the filaments subsequent to stretching in the presence of an aqueous solution of a water-soluble salt which is a coagulant for cellulose xanthate, said solution having an ion molality within the limits defined by the curves AB and CD of the graph shown as Figure 4 in the accompanying drawings and the pH at the point on the ordinate of said graph corresponding to said ion molality.

11. In the process for the production of a regenerated cellulose yarn which comprises extruding viscose filaments into a coagulating bath which will precipitate the cellulose xanthate without substantially converting it to regenerated cellulose, drawing said filaments from said bath, stretching said filaments and regenerating said filaments to regenerated cellulose, the improvement which comprises the step of swelling the filaments subsequent to stretching and prior to regeneration in the presence of an aqueous solution of a water-soluble salt which is a coagulant for cellulose xanthate, said solution having an ion molality within the limits defined by the curves AB and CD of the graph shown as Figure 4 in the accompanying drawings and the pH at the point on the ordinate of said graph corresponding to said ion molality.

12. In the process for the production of a regenerated cellulose yarn which comprises extruding viscose filaments into a coagulating bath which will precipitate the cellulose xanthate without substantially converting it to regenerated cellulose, drawing said filaments from said bath, stretching said filaments and regenerating said filaments to regenerated cellulose, the improvement which comprises the step of swelling the filaments subsequent to stretching and simultaneously with regeneration in the presence of an aqueous solution of a water-soluble salt which is a coagulant for cellulose xanthate, said solution having an ion molality within the limits defined by the curves AB and CD of the graph shown as Figure 4 in the accompanying drawings and the pH at the point on the ordinate of said graph corresponding to said ion molality.

13. In the process for the production of a regenerated cellulose yarn which comprises extruding viscose filaments into a coagulating bath which will precipitate the cellulose xanthate without substantially converting it to regenerated cellulose, drawing said filaments from said bath, stretching said filaments and regenerating said filaments to regenerated cellulose, the improvement which comprises the step of swelling the filaments subsequent to stretching in the presence of an aqueous solution of a water-soluble salt which is a coagulant for cellulose xanthate, said solution having an ion molality within the limits defined by the curves EF and GH of the graph shown as Figure 4 in the accompanying drawings and the pH at the point on the ordinate of said graph corresponding to said ion molality.

14. In the process for the production of a regenerated cellulose yarn which comprises extruding viscose filaments into a coagulating bath which will precipitate the cellulose xanthate without substantially converting it to regenerated cellulose, drawing said filaments from said bath, stretching said filaments and regenerating said filaments to regenerated cellulose, the improve-

ment which comprises the step of swelling the filaments subsequent to stretching and prior to regeneration in the presence of an aqueous solution of a water-soluble salt which is a coagulant for cellulose xanthate, said solution having an ion molality within the limits defined by the curves EF and GH of the graph shown as Figure 4 in the accompanying drawings and the pH at the point on the ordinate of said graph corresponding to said ion molality.

15. In the process for the production of a regenerated cellulose yarn which comprises extruding viscose filaments into a coagulating bath which will precipitate the cellulose xanthate without substantially converting it to regenerated cellulose, drawing said filaments from said bath, stretching said filaments and regenerating said filaments to regenerated cellulose, the improvement which comprises the step of swelling the filaments subsequent to stretching and simultaneously with regeneration in the presence of an aqueous solution of a water-soluble salt which is a coagulant for cellulose xanthate, said solution having an ion molality within the limits defined by the curves EF and GH of the graph shown as Figure 4 in the accompanying drawings and the pH at the point on the ordinate of said graph corresponding to said ion molality.

16. In the process for the production of a regenerated cellulose yarn which comprises extruding viscose filaments into a coagulating bath which will precipitate the cellulose xanthate without substantially converting it to regenerated cellulose, drawing said filaments from said bath, stretching said filaments and regenerating said filaments to regenerated cellulose, the improvement which comprises the step of swelling the filaments subsequent to stretching in the presence of an aqueous solution of a water-soluble neutral salt which is a coagulant for cellulose xanthate, said solution having an ion molality of 1 to 4 and a pH of 7.

17. In the process for the production of a regenerated cellulose yarn which comprises extruding viscose filaments into a coagulating bath which will precipitate the cellulose xanthate without substantially converting it to regenerated cellulose, drawing said filaments from said bath, stretching said filaments and regenerating said filaments to regenerated cellulose, the improvement which comprises the step of swelling the filaments subsequent to stretching in the presence of an aqueous solution of a water-soluble neutral salt which is a coagulant for cellulose xanthate, said solution having an ion molality of 2 to 3 and a pH of 7.

18. In the process for the production of a regenerated cellulose yarn which comprises extruding viscose filaments into a coagulating bath which will precipitate the cellulose xanthate without substantially converting it to regenerated cellulose, drawing said filaments from said bath, stretching said filaments and regenerating said filaments to regenerated cellulose, the improvement which comprises the step of swelling the filaments subsequent to stretching in the presence of an aqueous solution having a pH of 7 and an ion molality of from 1 to 4 and consisting of water and sodium sulfate, the latter being present in an amount of from 9% to 13% by weight of the solution.

19. In the process defined in claim 1 wherein the aqueous swelling solution contains a mixture of water-soluble salts.

20. In the process defined in claim 5 wherein

the aqueous swelling solution contains a mixture of water-soluble salts.

21. In the process defined in claim 1 wherein the aqueous swelling solution contains an alkali hydroxide when said solution has a pH above 7.

22. In the process defined in claim 5 wherein the aqueous swelling solution contains an alkali hydroxide when said solution has a pH above 7.

LINTON G. RAY, JR.

#### REFERENCES CITED

The following references are of record in the file of this patent:

#### UNITED STATES PATENTS

| Number    | Name          | Date          |
|-----------|---------------|---------------|
| 1,930,803 | Harrison      | Oct. 17, 1933 |
| 2,297,746 | Charch et al. | Oct. 6, 1942  |
| 2,412,969 | Cramer        | Dec. 24, 1946 |